

T. H. MATHIAS.

PROCESS OF ELIMINATING PIPES AND SEGREGATED METAL FROM INGOTS.

APPLICATION FILED MAR. 7, 1914. RENEWED APR. 20, 1918.

1,286,379.

Patented Dec. 3, 1918.

Fig. 1.



Fig. 2.



Fig. 3.



Fig. 4.



Fig. 5.



Fig. 7.



Fig. 6.



Fig. 9.



Fig. 8.



Fig. 10.



Witnesses:

J. M. Ellsworth  
W. H. Brewster

Inventor

Thomas H. Mathias  
By his Attorney  
Alfred Wilkinson.

# UNITED STATES PATENT OFFICE.

THOMAS H. MATHIAS, OF BUFFALO, NEW YORK, ASSIGNOR TO LACKAWANNA STEEL COMPANY, OF LACKAWANNA, NEW YORK, A CORPORATION OF NEW YORK.

## PROCESS FOR ELIMINATING PIPES AND SEGREGATED METAL FROM INGOTS.

1,286,379.

Specification of Letters Patent.

Patented Dec. 3, 1918.

Application filed March 7, 1914, Serial No. 823,058. Renewed April 20, 1918. Serial No. 229,871.

To all whom it may concern:

Be it known that I, THOMAS H. MATHIAS, a citizen of the United States, residing at Buffalo, in the county of Erie and State of New York, have invented new and useful Improvements in Processes for Eliminating Pipes and Segregated Metal from Ingots, of which the following is a specification.

My invention relates to the elimination of the pipe and the segregated metal from the billet or bloom to produce better rails and consists in a new method of rolling down the ingot.

Pipes are formed in the ingot during teeming, the piping and segregation taking place as the metal solidifies and increasing as the solidifying advances. This pipe extends down into the ingot a greater or less distance from the upper and usually smaller end, and results in a defect in the bar rolled from that piped portion, which is particularly dangerous when the bar is a rail. To avoid the production of such defective rails, the piped end is cropped, but this involves waste, and, entirely to remove the piped portion, would involve such great waste that it is never done, so that more or less piped rails are always produced.

Attempts have been made and processes suggested for rolling the ingot butt-end first before the interior is hardened, whereby the molten metal is forced toward the smaller end more or less filling the pipe, but such attempts have never proved entirely successful, owing to certain practical defects. These defects I believe I have overcome, and I have succeeded in eliminating the pipe and the segregated metal with a trifling waste, by a practical and economical process.

My process consists in rolling the ingot butt-end first and applying the pressure equally and uniformly to all four sides. This is done between a pair of rolls in which the grooves are so shaped that each roll applies pressure to two adjacent sides of the ingot with the result that the only openings between the rolls through which metal can be forced out to form fins is at the diagonally opposite corners. At the next pass

the relation of the billet to the rolls is changed so that the openings between the rolls come at the other pair of diagonally opposite corners and the fins starting at the first pass are rolled out in the second. This shifting, or change in relation, is continued in the successive passes throughout the entire rolling operation.

This formation of fins has been a serious, if not fatal, objection to all the processes for rolling out the pipes with which I am acquainted, and it will be understood that if such fins are formed in reducing the ingot they must be removed in some way which would be expensive, for if not they would be rolled out in the finished bar, forming seams, etc.

In the drawing forming a part of this description, Figure 1 is a longitudinal section of the ingot as originally cast. Fig. 2 is an elevation of a desirable form of rolls, Figs. 3, 4, 5 and 6 show the ingot in longitudinal section and the rolls in cross section to illustrate the steps of the rolling in which the pipe is rolled out. Figs. 7, 8, 9 and 10 are sections respectively of Figs. 3 to 6 to illustrate the change in relation of the ingot and the rolls whereby the fins are rolled out.

In the drawing 1 and 2 indicate respectively the upper and lower rolls; 4 and 5, respectively the upper and lower end of the ingot; and 6, the pipe. The ingot is cast in the tapering form shown to make stripping from the mold easy but my process could be applied to straight ingots as well. In every case however the ingot must be rolled butt first, that is, the pressure be applied from the lower end toward the upper, simultaneously on all four sides to force the hot soft metal of the interior toward the upper end to fill the pipe cavity, carrying with it the segregated metal surrounding said cavity. The procedure is best indicated in Figs. 3, 4, 5 and 6. As soon as the exterior of the ingot is sufficiently set and the ingot can be handled, the mold is stripped therefrom and the ingot transferred to the rolls. As a preliminary step I prefer to pass the ingot through the rolls once, small end first, to

eliminate the fin formed around the bottom edge between the mold and the stool, but this is not an essential part of my process.

The ingot is then passed through the rolls 5 butt or bottom end first several times, say four to ten, as may be desired whereby the hot, molten or soft metal is forced toward the small end until what is left of the pipe and practically all the segregated metal is 10 forced to the very end which is then cropped, this being merely a trifle as compared to the size of the crop and according to common practice. Thus not only are the pipe and the segregated metal entirely eliminated but 15 a great saving is effected in the amount cropped.

An essential feature of my process is the prevention or elimination of fins and this is important, for the presence of fins would 20 reduce the value of the ingot so far as to counterbalance any advantages. This is effected by applying the pressure to all sides of the ingot simultaneously, but by two surfaces, each continuous, and each applying 25 the pressure to two adjacent sides and reversing the relation of the ingot to the rolls at each successive pass.

This will be understood by reference to Figs. 7 and 8. A groove is formed in the 30 upper roll, of which the two surfaces, *a*, *b*, are arranged at a right angle to each other. Preferably and to make rolling easier, neither of these surfaces should be at a right angle to the roll axis, but each arranged at less than a right angle thereto. These angles may be similar, or one greater and the other less as may be desired. In 35 the form of rolls shown, the angle between the surface *b* and the longitudinal axis of the roll is the greater and approaches a right angle, but the angle between surface *a* and the axis is much less. Roll 2 is correspondingly formed with surfaces *a'*, *b'*. Between the pairs of surfaces are the corners *c*, *c'* of 40 rather large radius. Thus the pressure will be applied to the four sides by the two rolls, and, there being only two openings between the rolls, fins can be formed only at the ingot corners *d* and *d'*. But at the next 45 pass the relation of the corners and the openings are reversed, the ingot being shifted a quarter turn around its longitudinal axis bringing the corners *d*, *d'* at the corners *f*, *f'* where the rudimentary fins will be rolled out, and fins begin to be formed 50 on corners *e*, *e'* which in their turn are rolled out in the third pass, etc.

I have spoken of shifting the ingot but in practice I prefer instead to change the 55 position of the openings and the corners in the successive stands of rolls. Referring to Fig. 8, this change will be understood; it will be seen that the ingot corners *d*, *d'*

which were at at openings in the rolls of Fig. 7 are now at the corners *f*, *f'* and the 60 openings will tend to form fins on the corners *e*, *e'*.

Furthermore I prefer to arrange my rolls in tandem, for, to turn the ingot around end for end at each pass, would involve too 70 much labor, waste time and permit the cooling of the ingot.

Changes may be introduced into my process without departing from the spirit thereof, for instance it is not necessary that there 75 should be a shift in the bar at every successive pass, but merely a sufficiently frequent shift, or change in its relation to the rolls, to eliminate the fins.

Having described my invention, I claim,— 80

1. The method of rolling down ingots substantially to eliminate the pipe and segregated metal, consisting in passing the ingot through rolls a plurality of times butt-end first and applying the pressure equally 85 and uniformly to all four sides.

2. The method of rolling down ingots substantially to eliminate the pipe and to force all segregated metal to the extreme end of the ingot, which consists in passing 90 the ingot through the rolls a plurality of times lower end first, the grooves in the rolls 95 being shaped so that each roll shall apply pressure to two adjacent sides of the ingot and one pair of diagonally opposite corners 100 of the ingot shall correspond with the joints between the rolls, and during some of the passes changing the relation of the ingot and the rolls so that each roll shall engage with different surfaces and the other pair 105 of opposite corners of the ingot shall correspond with the joints between the rolls.

3. The method of rolling down ingots substantially to eliminate the pipe, which consists in passing the ingot between rolls 110 lower end first a plurality of times while the ingot interior is still molten, the passes in the rolls being formed each with two continuous surfaces having a corner of large radius between them, the two surfaces on 115 each roll being arranged substantially at a right angle to each other and each surface at less than a right angle to the roll axis, said two surfaces being adapted to apply pressure to two adjacent sides of the ingot, and at each successive pass turning the ingot about its longitudinal axis with relation to the rolls, so that at one pass one pair of diagonally opposite ingot corners shall be received in the roll corners, and, at the next 120 pass, the other pair of diagonally opposite ingot corners.

4. The method of rolling down ingots substantially to eliminate the pipe and to force all the segregated metal to the extreme 125 end of the ingot, which consists in passing

the ingot through the rolls a plurality of times lower end first, and applying the pressure equally and uniformly to all four sides of the ingot by means of a pair of rolls each 5 having a groove so shaped that each roll shall apply pressure to two adjacent sides of the ingot.

In testimony whereof I have signed my name to this specification in the presence of two subscribing witnesses.

THOMAS H. MATHIAS.

Witnesses:

JOSEPH E. DONNELLY,  
WALTER J. BRYAN.

Copies of this patent may be obtained for five cents each, by addressing the "Commissioner of Patents, Washington, D. C."